

## UNITED STATES PATENT OFFICE

2,015,864

## PROCESSING OF TEXTILES

Adalbert Müller and Theodor Stenzinger, Augsburg, Germany, assignors to Erba Aktiengesellschaft, Fabrik Chemischer Produkte, Zurich, Switzerland, a corporation of Switzerland

No Drawing. Application October 18, 1932, Serial No. 638,345. In Germany December 17, 1931

4 Claims. (Cl. 91—68)

The invention relates to processes of treating textiles and similar materials, and it particularly relates to a method of incorporating waxy or fatty materials and other water insoluble materials in textiles, yarns or fabrics.

An object of the present invention is to provide a process whereby water insoluble materials may be incorporated in textiles and similar materials for softening, waterproofing, sizing, lustre-finishing and other finishing, with assurance that the loading material will be substantially permanently incorporated in the body of the fiber or structure of the textile.

Another object is to provide a process whereby water insoluble materials may be incorporated in textiles and similar materials for softening, waterproofing, sizing, lustre-finishing and other finishing, with assurance that the loading material will be substantially permanently incorporated in the body of the fiber or structure of the textile by treating with emulsions or colloidal dispersions which admits of the possibility of utilizing very dilute emulsions or colloidal dispersions containing the water insoluble material.

Another object is to provide improved colloidal dispersions or emulsions, which are particularly adapted for loading or filling textile materials, as for example to waterproof them.

Another object is to provide improved waterproof textile materials which contain relatively small quantities of the water-proofing or fatty substances, substantially permanently absorbed inside of the fiber or inside of the structure of the textile itself.

Other objects are in part obvious and will be in part pointed out hereinafter.

If a textile or similar material having an electrical charge, for example a negative charge, is treated with a colloidal dispersion or emulsion, the suspended particles of which have an opposite or positive charge, it has been found that the dispersed particles of the colloidal dispersion or emulsion will incorporate themselves with and penetrate into the structure of the textile, fabric, or other similar material, even though the emulsion be very dilute. Satisfactory incorporation and consequently desirable waterproofed or finished textiles are obtained without using a highly concentrated bath.

According to the present invention it is desirable to subject the textile materials to treatment in the colloidal emulsions or dispersions for a longer period of time than has previously been the case, but this increase in exposure is over-balanced by the many other advantages

accruing from the utilization of a relatively dilute solution.

Usually, textiles have a negative charge, and in such case a positively charged colloid dispersion would be employed. However, if the textile has a positive charge, a negatively charged dispersion should preferably be employed. The negatively charged textile material may be changed into a positively charged one by treating it with suitable acids, salts and dyes. This change may for example be accomplished by subjecting it to suitable dyeing processes.

Among the textile materials wool, cotton, silk, artificial silk, linen and the like may be treated by the present invention. Materials in non-spun state, as for instance top, or woven or knitted yarn may also be treated. If desired, paper, leather, fur and other materials may also be similarly processed. The emulsion may contain colloidally dispersed fats, waxy materials, oleaginous substances and other water-proofing or water insoluble materials. Other substances such as resin, caoutchouc, sulphur, asphalt and the like may also be employed in the emulsions.

The following are several illustrative examples of preferred modes of carrying out the process of the present invention, to which the invention is not to be limited:

(1.) 1 kg. of an emulsion containing about 25% cocoa fat and a small amount of acetic acid, and the dispersed phase of which is positively charged, is mixed with 200 ltrs. of water. 10 kg. knitted cotton are treated with this solution on a mechanical or hand winch for about 10 to 15 minutes at a temperature of 120° F. At the end of this time the bath will clarify. After finishing, the cotton material will possess the desired degree of softness.

If a negatively charged cocoa fat emulsion is employed, that is one having the same charge as the fabric, the same effect may only be obtained with an emulsion having 4 or 5 times the above concentration.

(2.) 30 kg. of woollen yarn are dyed with the aid of sulphuric acid. After rinsing, the yarn will still contain considerable quantities of acid and consequently will be positively charged. The material is then agitated in 2000 ltrs. of a bath containing 2.5 kg. of a concentrated paraffin emulsion, said emulsion containing about 30% paraffin. After a processing for 15 to 20 minutes at 90 to 110° F. the bath will become completely clear. The treated yarns are then dehydrated by centrifuging and then dried, after which they may be easily spun.

(3) 50 kg. of woollen yarn are dyed in an Esser apparatus and then rinsed.

2.5 kg. of a concentrated paraffin emulsion containing sufficient quantities of aluminium salt to charge it positively are mixed with 3000 liters of water. The dyed and rinsed wool is then treated with this mixture for about 30 minutes at a temperature of from 110 to 120° F. after which the liquid mixture will become perfectly clear.

10 After the liquid has been removed the woollen yarn is washed with a spray of cold water and centrifuged and dried. Very good impregnation is thus obtained.

(4) 0.3 kg. of an emulsion containing 10% wax and 10% of a fatty acid are mixed with 300 liters of water. Then, 0.2 liter of a solution of aluminium formate bearing a strength of 8° Bé. are added to this liquor. 10 kg. of an artificial silk material are treated in this bath on an open width 15 scourer for about 10 to 15 minutes at a temperature of between 60 and 70° F. The bath will clarify. After the drying the artificial silk material will be very water-repellent.

The incorporation of the fatty material, according to the present invention in a textile material may form part of an impregnating, softening, finishing, or other textile treating processes. The present invention has many advantages over processes which treat textiles with emulsions having the same charge as the textile, since in these processes, it is necessary to use a relatively concentrated bath, said bath containing about 2 to 30 5% of a concentrated emulsion having for instance 30% water insoluble substances.

35 Textile materials, when treated with emulsions of this character, are only mechanically penetrated by the liquor of the bath and retain, when pressed or squeezed out, 50 to 100% of their own weight of the liquid in the bath. In these cases instead of the water-proofing or fatty materials 40 being incorporated inside of or absorbed by the fiber or structure of textile, they will be deposited on the surface upon evaporation of the water from the emulsion upon drying.

45 With 100 liters of the bath containing for example 2% of a concentrated emulsion, as above described, about 3 kg. of textile material may be treated. In other words, 3 kg. of goods must be treated with 2 kg. of the concentrated emulsion or with an amount of the emulsion equivalent to 50 66% of the weight of the material treated.

According to the present invention the textiles are treated with at most an amount of emulsion equivalent to 10% by weight of the materials being treated. Thus, 3 kg. of the material may be treated with 100 liters of a bath containing 55 0.3% of the emulsion.

The treatment of the material by the bath is carried out for a rather extended time, generally for 60 10 to 30 minutes.

According to the process of the present invention the time of treatment of the materials in all the apparatus used, in which the materials may be subjected to treatment, as for example the reeling vat, the washing-machine, or the vessel, is preferably continued for a suitably extended period. The temperature of the bath may be between 70 and 180° F. according to the material being treated. Materials which may be 65 readily affected, such as artificial silk, are treated preferably at lower temperatures. With higher temperatures the extraction of the emulsion will be accelerated.

Because of the opposite charges of the textile material and the emulsion, it appears that the 70 75

combination between the textile and the colloidally dispersed material is of the same character as takes place during the flocculation and coagulation as will result upon the mixture of two oppositely charged colloidal solutions or dispersions. This process is much slower than ordinary precipitation processes involving the 5 ionic reactions and it is necessary to carry out the treatment until the desired amount of combination between the textile and the colloidal material has been obtained.

The combination between the textile and the colloidal waxy and fatty particles is such that the water-proofing material will be retained in the textile even though it be subjected to drastic 15 washing or other operations over long periods of time.

Although it is desirable to obtain a complete extraction of the emulsion and a resultant clarity of the bath, the desirable water-proofing action 20 between the textile and the colloid will be obtained even if the bath does not clarify.

The emulsions of the present invention may be conveniently prepared with soaps, sulphonated oils or fats or other proper fatty derivatives, 25 aromatic sulphonic acids, sulphonated mineral oils and the like. Further the emulsification may be assisted by colloidal substances, such as proteins, albumins, casein, glue, starch, cellulosic materials, sulphite waste liquor and the like. 30 These emulsions will possess a negative charge and may be satisfactorily utilized to treat positively charged textiles.

Positively charged emulsions may be obtained from such negatively charged emulsions by the 35 addition of substances giving a positive charge to the dispersed phase. Such substances are free acids as for instance hydrochloric acid, sulphuric acid, formic acid, acetic acid, lactic acid and tartaric acid or salts having an acid reaction. 40 Salts of polyvalent metals, such as salts of aluminium, iron, zinc, copper and the like, as well as positively charged hydrosols for instance aluminium hydroxide may also be employed. The positive charging of the dispersed phase of the emulsion may be done by adding discharging substances to the dilute or concentrated negatively charged emulsion. In addition, positive emulsions may be directly produced by homogenizing the water insoluble substance with an aqueous 45 solution of the emulsifying agent and of the discharging substance.

If the discharge-causing material is added to concentrated emulsions and dispersions before dilution, it is possible to incorporate in the emulsions a greater amount of the discharge-causing material. As a result it is possible to obtain a greater charge upon each particle. By regulating the charge upon the colloidal particles and/or by also regulating the charge upon the textile 55 or similar material being treated, it is possible to regulate the affinity of these colloidal particles for the textile materials.

The present application relates to similar subject matter as the co-pending application, Serial No. 562,608, filed September 12, 1931, on Stable emulsions and processes for their production.

The claims of the present application are specifically directed to waterproof textiles with a negative charge caused by a positively charged 70 emulsion, which process may be carried out in a one bath operation, eliminating the necessity of utilizing a two bath process with its attendant disadvantages.

The subject matter disclosed and referred to in 75

the present application but not claimed herein is covered in the co-pending applications, Serial No. 659,506 filed March 3, 1932 and Serial No. 745,755 filed September 27, 1934.

5 It is to be understood that the many alterations and modifications may be made in the present application without departing from the invention set forth and described and it is to be understood that the examples given have merely been cited by 10 way of illustration and not by way of limitation and it is intended by the present application to cover the invention in its broadest aspects.

What we claim is:

1. A process of waterproofing textiles with wa- 15 ter insoluble, oily, waxy and fatty materials from aqueous emulsions thereof, which comprises pro- viding the textile with a negative charge, prepar- ing an emulsion of said water insoluble materials in which the emulsified or disperse phase is posi- 20 tively charged and then immersing the textiles in said bath to cause them to absorb the disperse phase from the bath by reason of their opposite charge.

2. A process of waterproofing textiles with a 25 water insoluble material selected from the class consisting of cocoa fat, olive oil and paraffin,

which comprises providing the textile with a nega- 5 tive charge, preparing a dilute aqueous emulsion containing said water insoluble material in the disperse phase and having a positive charge, and immersing the textiles in said bath to cause said textiles to absorb said water insoluble material from the bath by reason of their opposite charge.

3. A process of water proofing textiles with paraffin which comprises providing the textiles with a negative charge, preparing a diluted emul- 10 sion containing the paraffin in the disperse phase and positively charged and then immersing the textiles in the dilute bath to absorb the paraffin therefrom by reason of the opposite charge.

4. A process of water proofing textiles with 15 paraffin and an aluminum compound which com- prises providing the textiles with a negative charge, preparing a diluted emulsion containing the paraffin in the disperse phase and containing 20 an aluminum compound and positively charged and then immersing the textiles in the dilute bath to absorb the paraffin therefrom by reason of the opposite charge.

ADALBERT MÜLLER. 25  
THEODOR STENZINGER.